

July 14, 1959

R. SMITH

2,894,867

METHOD OF PRODUCING TRANSFORMATION HARDENABLE STAINLESS  
STEEL AND ARTICLES PRODUCED THEREFROM

Filed July 11, 1957

FIG. 1.



FIG. 2.



INVENTOR  
RAYMOND SMITH

By: Donald G. Dalton  
Attorney

1

2,894,867

**METHOD OF PRODUCING TRANSFORMATION HARDENABLE STAINLESS STEEL AND ARTICLES PRODUCED THEREFROM**

Raymond Smith, Pittsburgh, Pa., assignor to United States Steel Corporation, a corporation of New Jersey

Application July 11, 1957, Serial No. 671,213

12 Claims. (Cl. 148—21.55)

This invention relates to production of transformation hardenable stainless steel and more particularly to austenitic stainless steel which is hardenable by low temperature transformation.

In the construction of modern aircraft, guided missiles and the like, there is need for steels having good high temperature and corrosion resistance properties which can be fabricated in the soft austenitic condition and later transformed to the desired minimum hardness of Rockwell C39 or a minimum tensile strength of 180,000 p.s.i. Steels which harden by precipitation are unsuitable for prolonged use at temperatures approaching or above the hardening temperature due to their tendency to soften.

I have found that these desired properties can be produced by the proper heat treatment of a steel containing about 15 to 18% chromium, about .55 to 1.75% vanadium together with carbon and nickel within certain critical limits as more fully described hereinafter.

Such steel has the following general composition limits:

|           | Percent      | 35 |
|-----------|--------------|----|
| Carbon    | .03 to .30   |    |
| Manganese | .50 to 2.0   |    |
| Silicon   | .20 to 1.50  |    |
| Nickel    | 3.0 to 7.5   |    |
| Chromium  | 15.0 to 18.0 | 40 |
| Vanadium  | .55 to 1.75  |    |

balance substantially iron and other elements in amounts which do not adversely affect the properties.

Within such limits the ferrite formers and austenite formers must be balanced to provide an  $M_s$  point in the steel which is below room temperature and preferably between about 0° F. and —50° F. The vanadium content

2

should be kept below about 1.75% since higher quantities result in the steel having considerable quantities of delta ferrite so that hot working of the steel is quite troublesome.

The heat treatment comprises quenching the steel from a temperature of 1700 to 2100° F. to a soft austenitic condition followed by transforming the steel to an essentially martensitic structure by cooling it to a low temperature, preferably to about —100° F. or below. Following such transformation, the steels may be tempered in the range of 700 to 1100° F. and preferably at about 800° F. to produce a tempered martensitic structure therein.

Figures 1 and 2 of the accompanying drawing which are graphs wherein the ordinates denote the percentage of chromium and the abscissas the sum of the product of 30 times the percentage of carbon content plus the percentage of nickel. The shaded areas ABCD and  $A_1B_1C_1D_1$  represent the amounts of chromium and combined amounts of carbon and nickel which will give the desired results with the particular austenitizing treatment shown. Thus Figure 1 depicts the best composition for an 1800° F. austenitizing temperature and Figure 2 the composition requiring a 2000° F. austenitizing temperature. Steels having compositions falling to the right of the lines AB, and  $A_1B_1$  do not transform or harden to a satisfactory degree whereas those falling to the left of the lines CD, and  $C_1D_1$  transform and harden upon cooling to room temperature after annealing.

The following Table I lists the composition of a number of heats which are illustrative of the steels of my invention:

Table I

| Heat | O    | Mn   | P    | S    | Si  | Ni   | Cr    | V    | Sol. N <sub>2</sub> |
|------|------|------|------|------|-----|------|-------|------|---------------------|
| 1545 | .101 | .98  | .008 | .012 | .39 | 4.55 | 17.13 | 1.12 | .045                |
| 1542 | .117 | 1.01 | .007 | .014 | .43 | 5.29 | 15.66 | 1.18 | .041                |
| 1549 | .151 | .90  | .009 | .008 | .36 | 4.48 | 16.83 | 1.12 | .043                |
| 1550 | .198 | .88  | .008 | .010 | .39 | 4.46 | 16.10 | 1.12 | .043                |
| 1561 | .23  | 1.02 | .007 | .016 | .48 | 3.81 | 16.45 | 1.08 | .051                |
| 1564 | .26  | .98  | .007 | .019 | .39 | 4.06 | 16.30 | 1.03 | .049                |
| 1134 | .058 | 1.08 | .010 | .027 | .47 | 6.56 | 16.78 | 1.07 | .031                |
| 1486 | .076 | 1.04 | .009 | .019 | .47 | 5.57 | 16.96 | 1.15 | .025                |
| 1177 | .044 | 1.00 | .011 | .022 | .66 | 6.06 | 17.30 | 1.15 | .045                |
| 1504 | .077 | 1.00 | .010 | .020 | .54 | 5.46 | 18.16 | 1.05 | .13                 |
| 1562 | .20  | 1.03 | .008 | .016 | .72 | 4.31 | 16.15 | .60  | .048                |

The effect of various annealing temperatures on these is shown in the following Table II.

Table II

| Heat | 15 Min. 1,800 F., W.Q. |                                | 15 Min. 1,900 F., W.Q. |                                | 15 Min. 2,000 F., W.Q. |                                | 15 Min. 2,050 F., W.Q. |                                |
|------|------------------------|--------------------------------|------------------------|--------------------------------|------------------------|--------------------------------|------------------------|--------------------------------|
|      | Rockwell Hardness      |                                | Rockwell Hardness      |                                | Rockwell Hardness      |                                | Rockwell Hardness      |                                |
|      | Annealed               | 2 Hr. —110 F.<br>+2 Hr. 800 F. | Annealed               | 2 Hr. —110 F.<br>+2 Hr. 800 F. | Annealed               | 2 Hr. —110 F.<br>+2 Hr. 800 F. | Annealed               | 2 Hr. —110 F.<br>+2 Hr. 800 F. |
| 1545 | C33.5                  | C40.0                          | B96.0                  | C43.5                          | B93.5                  | C39.5                          | B94.0                  | C45.0                          |
| 1542 | C38.5                  | C44.0                          | B96.0                  | C45.0                          | B95.0                  | C44.0                          | B95.0                  | C43.0                          |
| 1549 | C43.5                  | C43.0                          | B97.0                  | C46.5                          | B92.5                  | C42.5                          | B94.0                  | C45.0                          |
| 1550 | C31.0                  | C47.0                          | B99.0                  | C47.0                          | B91.5                  | C45.0                          | B91.5                  | C47.0                          |
| 1561 | C44.0                  | C47.5                          | C34.0                  | C46.0                          | C21.5                  | C46.0                          | B95.5                  | C42.0                          |
| 1564 | C38.5                  | C47.5                          | C36.0                  | C47.0                          | B98.5                  | C40.5                          | B98.5                  | C36.5                          |

The following Table III lists certain steels which were martensitic as annealed.

Table III

| Heat  | C    | Mn   | P    | S    | Si  | Ni   | Cr    | V    | Sol. N <sub>2</sub> |
|-------|------|------|------|------|-----|------|-------|------|---------------------|
| 1255  | .034 | 1.02 | .006 | .030 | .48 | 5.02 | 16.93 | 1.02 | .034                |
| 1220  | .070 | .96  | .008 | .030 | .44 | 5.58 | 15.98 | .99  | .030                |
| 1399  | .070 | 1.03 | .010 | .030 | .48 | 5.87 | 15.95 | 1.03 | .027                |
| 1501  | .053 | 1.00 | .008 | .020 | .54 | 5.05 | 17.40 | 1.05 | .038                |
| 1241* | .081 | 1.04 | .006 | .032 | .51 | 5.65 | 16.68 | 1.99 | -----               |

Typical steels which were austenitic as annealed and not hardenable are listed in the following Table IV.

Table IV

| Heat  | C    | Mn   | P    | S    | Si  | Ni   | Cr    | V    | Sol. N <sub>2</sub> |
|-------|------|------|------|------|-----|------|-------|------|---------------------|
| 1218  | .068 | .88  | .008 | .032 | .47 | 6.51 | 16.91 | .99  | .041                |
| 1136  | .110 | 1.00 | .012 | .026 | .44 | 6.50 | 15.75 | 1.02 | .027                |
| 1178  | .086 | 1.00 | .012 | .026 | .74 | 6.07 | 17.45 | 1.12 | .036                |
| 1403  | .093 | 1.10 | .010 | .025 | .50 | 6.44 | 16.36 | 1.03 | .032                |
| 1189  | .086 | 1.00 | .011 | .027 | .67 | 6.01 | 16.45 | .51  | -----               |
| 1190  | .13  | 1.58 | .010 | .026 | .65 | 5.89 | 16.44 | .49  | -----               |
| 1244* | .078 | 1.00 | .006 | .027 | .49 | 6.68 | 17.63 | 1.99 | -----               |

\*Showed 10-15% delta ferrite in annealed condition.

A preferred embodiment of the steel of my invention for developing hardness value in excess of C-45 or tensile strengths in excess of 220,000 p.s.i. contains

|           | Percent      |
|-----------|--------------|
| Carbon    | .15 to .26   |
| Manganese | .75 to 1.20  |
| Silicon   | .35 to .75   |
| Nickel    | 3.40 to 5.6  |
| Chromium  | 16.0 to 17.3 |
| Vanadium  | .60 to 1.20  |

Steels of this composition should fall within the area A<sub>1</sub>B<sub>1</sub>C<sub>1</sub>D<sub>1</sub> of Figure 2 and annealed in the range of 1975 to 2025° F., i.e. at about 2000° F., transformed by cooling to about -110° F. Thereafter such steels may be tempered in the range of 700 to 1100° F. and preferably at about 800° F. to produce the maximum properties. As indicated, such steels will have a Rockwell C value in excess of 45 or tensile strengths in excess of 220,000. Moreover, they are soft and ductile in the annealed condition.

If lower strengths and hardnesses are desired with attendant improvement in ductile properties the following composition having lower carbon and higher nickel contents in conformity with the area ABCD of Figure 1 of the drawing may be used:

|           | Percent     |
|-----------|-------------|
| Carbon    | .04 to .12  |
| Manganese | .75 to 1.20 |
| Silicon   | .35 to .75  |
| Nickel    | 4.7 to 7.0  |
| Chromium  | 15. to 17.8 |
| Vanadium  | .60 to 1.20 |

Such steel should be annealed at a temperature in the range of about 1775 to 1825° F. and quenched to a soft workable austenitic condition. Thereafter it may be hardened by transforming at low temperatures, i.e. below about -100° F. following which may be tempered at about 800° F. is desired.

While I have shown and described several specific embodiments of my invention, it will be understood that these embodiments are merely for the purpose of illustration and description and that various other forms

may be devised within the scope of my invention, as defined in the appended claims.

I claim:

1. Stainless steel characterized by being transformable to a hard martensitic structure by sub-zero treatment from a soft austenitic structure in the annealed condition which can be tempered to improve the ductility thereof, said steel containing

|           | Percent      |
|-----------|--------------|
| Carbon    | .03 to .30   |
| Manganese | .50 to 2.00  |
| Silicon   | .20 to 1.5   |
| Nickel    | 3.0 to 7.5   |
| Chromium  | 15.0 to 18.0 |
| Vanadium  | .55 to 1.75  |

the ferrite formers being balanced to provide an M<sub>s</sub> temperature between about 0° F. and -50° F. with the remainder iron and other elements in amounts which do not adversely affect the properties.

2. Stainless steel characterized by being transformable to a hard martensitic structure from a soft austenitic structure in the annealed condition which can be tempered to improve the ductility thereof, said steel containing

|           | Percent      |
|-----------|--------------|
| Carbon    | .15 to .26   |
| Manganese | .75 to 1.2   |
| Silicon   | .35 to .75   |
| Nickel    | 3.4 to 5.6   |
| Chromium  | 16.0 to 17.3 |
| Vanadium  | .6 to 1.2    |

the ferrite formers and the austenite formers being balanced to provide an M<sub>s</sub> temperature between about 0° F. and -50° F. with the balance iron and other elements in amounts which do not adversely affect the properties.

3. Stainless steel characterized by being transformable to a hard martensitic structure from a soft austenitic structure in the annealed condition which can be tempered to improve the ductility thereof, said steel containing

|           | Percent      |
|-----------|--------------|
| Carbon    | .04 to .12   |
| Manganese | .75 to 1.2   |
| Silicon   | .35 to .75   |
| Nickel    | 4.7 to 7.0   |
| Chromium  | 15.0 to 17.8 |
| Vanadium  | .6 to 1.2    |

the ferrite formers and the austenite formers being balanced to provide an M<sub>s</sub> temperature between about 0° F. and -50° F. with the balance iron and other elements in amounts which do not adversely affect the properties.

4. Thermally hardened articles composed of stainless steel containing

|           | Percent      |
|-----------|--------------|
| Carbon    | .03 to .30   |
| Manganese | .50 to 2.0   |
| Silicon   | .20 to 1.5   |
| Nickel    | 3.0 to 7.5   |
| Chromium  | 15.0 to 18.0 |
| Vanadium  | .55 to 1.75  |

wherein the austenite and ferrite formers are balanced to provide an M<sub>s</sub> temperature between about 0° F. and -50° F. with the balance iron and other elements in amounts which do not adversely affect the properties, said steel having been annealed at a temperature in the range of 1700° to 2100° F. and quenched to provide a soft austenitic readily formable structure and thereafter

hardened by cooling it to below about  $-100^{\circ}$  F. to transform it to a hard martensitic structure.

5. Thermally hardened steel articles characterized by a tensile strength in excess of 220,000 p.s.i. composed of stainless steel containing

|           | Percent      |
|-----------|--------------|
| Carbon    | .15 to .26   |
| Manganese | .75 to 1.20  |
| Silicon   | .35 to .75   |
| Nickel    | 3.40 to 5.6  |
| Chromium  | 16.0 to 17.3 |
| Vanadium  | .6 to 1.2    |

wherein the austenite formers and ferrite formers are balanced to provide an  $M_s$  temperature between about 0 and  $-50^{\circ}$  F. and the chromium, nickel and carbon are within the area  $A_1B_1C_1D_1$  of the drawing, with the balance iron and other elements in amounts which do not adversely affect the properties, said steel having been annealed at a temperature in the range of 1975 to 2025° F. and quenched to provide a soft austenitic easily formable structure and thereafter hardened by cooling to below about  $-100^{\circ}$  F. to transform it to a hard martensitic structure.

6. Thermally hardened steel articles composed of stainless steel containing

|           | Percent      |
|-----------|--------------|
| Carbon    | .04 to .12   |
| Manganese | .75 to 1.20  |
| Silicon   | .35 to .75   |
| Nickel    | 4.7 to 7.0   |
| Chromium  | 15.0 to 17.8 |
| Vanadium  | .6 to 1.20   |

wherein the austenite formers and ferrite formers are balanced to provide an  $M_s$  temperature between about 0 and  $-50^{\circ}$  F. and the chromium, nickel and carbon are within the area ABCD of the drawing with the balance iron and other elements in amounts which will not adversely affect the properties, said steel having been annealed at a temperature in the range of 1775 to 1825° F. and quenched to provide a soft readily formable austenitic structure and thereafter hardened by cooling to below about  $-100^{\circ}$  F. to transform it to a hard martensitic structure.

7. A method of producing hardened stainless steel comprising making stainless steel containing

|           | Percent      |
|-----------|--------------|
| Carbon    | .03 to .30   |
| Manganese | .50 to 2.0   |
| Silicon   | .20 to 1.5   |
| Nickel    | 3.0 to 7.5   |
| Chromium  | 15.0 to 18.0 |
| Vanadium  | .55 to 1.75  |

the ferrite formers and the austenite formers being balanced to provide an  $M_s$  temperature between about 0 and  $-50^{\circ}$  F., with the balance iron and other elements in amounts which do not adversely affect the properties, annealing said steel at a temperature in the range of 1700 to 2100° F., quenching it to provide a soft austenitic readily formable structure and then cooling said annealed steel to below about  $-100^{\circ}$  F. to transform it to a hard martensitic structure.

8. A method of producing hardened stainless steel comprising making stainless steel containing

|           | Percent      |
|-----------|--------------|
| Carbon    | .15 to .26   |
| Manganese | .75 to 1.2   |
| Silicon   | .35 to .75   |
| Nickel    | 3.4 to 5.6   |
| Chromium  | 16.0 to 17.3 |
| Vanadium  | .6 to 1.2    |

wherein the austenite formers and ferrite formers are balanced to provide an  $M_s$  temperature between about 0 and  $-50^{\circ}$  F. and the chromium, nickel and carbon are within the area  $A_1B_1C_1D_1$  of the drawing, with the balance iron and other elements which do not adversely affect the properties, annealing said steel at a temperature in the range 1975 to 2025° F., quenching it to provide a soft readily formable austenitic structure and then cooling said annealed steel to below about  $-100^{\circ}$  F. to transform it to a hard martensitic structure.

9. A method of producing hardened stainless steel comprising making stainless steel containing

|           | Percent      |
|-----------|--------------|
| Carbon    | .04 to .12   |
| Manganese | .75 to 1.20  |
| Silicon   | .35 to .75   |
| Nickel    | 4.7 to 7.0   |
| Chromium  | 15.0 to 17.8 |
| Vanadium  | .6 to 1.2    |

wherein the austenite formers and ferrite formers are balanced to provide an  $M_s$  temperature between about 0 and  $-50^{\circ}$  F. and the chromium, nickel and carbon are within the area ABCD of the drawing, with the balance iron and other elements which do not adversely affect the properties, annealing said steel at a temperature in the range of 1775 to 1825° F. and quenching it to provide a soft readily formable austenitic structure, and then cooling said annealed steel to below about  $-100^{\circ}$  F. to transform it to a hard martensitic structure.

10. A method of producing articles of hardened stainless steel comprising making stainless steel containing

|           | Percent      |
|-----------|--------------|
| Carbon    | .03 to .30   |
| Manganese | .50 to 2.0   |
| Silicon   | .20 to 1.5   |
| Nickel    | 3.0 to 7.5   |
| Chromium  | 15.0 to 18.0 |
| Vanadium  | .55 to 1.75  |

the ferrite formers and the austenite formers being balanced to provide an  $M_s$  temperature between about 0 and  $-50^{\circ}$  F., with the balance iron and other elements in amounts which do not adversely affect the properties, annealing said steel at a temperature in the range of 1700 to 2100° F., quenching it to provide a soft austenitic readily formable structure, forming the desired articles therefrom and then cooling said annealed steel articles to below about  $-100^{\circ}$  F. to transform the steel thereof to a hard martensitic structure.

11. A method of producing articles of hardened stainless steel comprising making stainless steel containing

|           | Percent      |
|-----------|--------------|
| Carbon    | .15 to .26   |
| Manganese | .75 to 1.2   |
| Silicon   | .35 to .75   |
| Nickel    | 3.4 to 5.6   |
| Chromium  | 16.0 to 17.3 |
| Vanadium  | .6 to 1.2    |

65 wherein the austenite formers and ferrite formers are balanced to provide an  $M_s$  temperature between about 0 and  $-50^{\circ}$  F. and the chromium, nickel and carbon are within the area  $A_1B_1C_1D_1$  of the drawing, with the balance iron and other elements which do not adversely affect the properties, annealing said steel at a temperature in the range of 1975 to 2025° F., quenching it to provide a soft readily formable austenitic structure, forming the desired articles therefrom and then cooling said annealed steel articles to below about  $-100^{\circ}$  F. to transform the steel thereof to a hard martensitic structure.

12. A method of producing articles of hardened stainless steel comprising making stainless steel containing

|           | Percent      |
|-----------|--------------|
| Carbon    | .04 to .12   |
| Manganese | .75 to 1.20  |
| Silicon   | .35 to .75   |
| Nickel    | 4.7 to 7.0   |
| Chromium  | 15.0 to 17.8 |
| Vanadium  | .6 to 1.2    |

5 10

wherein the austenite formers and ferrite formers are balanced to provide an  $M_s$  temperature between about 0 and  $-50^{\circ}$  F. and the chromium, nickel and carbon are

within the area ABCD of the drawing, with the balance iron and other elements which do not adversely affect the properties, annealing said steel at a temperature in the range of 1775 to 1825° F. and quenching it to provide a soft readily formable austenitic structure, forming the desired articles therefrom, and then cooling said annealed steel articles to below about  $-100^{\circ}$  F. to transform the steel thereof to a hard martensitic structure.

References Cited in the file of this patent

UNITED STATES PATENTS

2,562,854 Binder July 31, 1951  
2,799,602 Lena July 16, 1957